

1

3,589,857

PROCESS OF BLEACHING TEXTILES  
Leo Thomas Murray, East Brunswick, N.J., assignor to  
Colgate-Palmolive Company, New York, N.Y.  
No Drawing. Filed Oct. 24, 1967, Ser. No. 677,745  
Int. Cl. D061 3/02

U.S. CL. 8—111

2 Claims

## ABSTRACT OF THE DISCLOSURE

Activator compounds for peroxide bleaching agents comprising alkyl and aryl chloroformates e.g., methyl chloroformate, ethyl chloroformate and phenyl chloroformate.

The present invention relates, in general, to compositions advantageously adapted for use in connection with fabric washing and bleaching operations and, in particular, to the provision of specific compounds and compositions for such purposes, said compositions being capable of providing an exceptionally high order of bleaching activity.

The utilization of bleaching agents as an adjunct to fabric washing operations is, of course, common practice if not a recognized necessity. Consequently, many of the detergent compositions currently available commercially contain predetermined amounts of bleaching agent as an essential ingredient; specific representatives of bleaching agents found to be suitable in this regard are well known in the art being extensively described in the published literature both patent and otherwise and include, for example, the chlorine bleaches such as the alkali metal hypochlorites; active oxygen-releasing peroxide compounds such as inorganic persalts e.g., the perborates, percarbonates, perphosphates, persilicates, persulfates, hydrogen peroxide, sodium peroxide and the like.

The peroxide type bleaching agents are, in general, preferred for use being found to be markedly superior as regards capability of providing a fabric having a softer hand, improved absorbency, permanence of whites and the like. In contradistinction, other types of bleaching agents currently enjoying relatively widespread commercial exploitation invariably yield fabrics having a pronounced tendency to develop spurious discoloration, e.g., yellowing. Moreover, fabric materials treated with bleach agents of this type, in many instances, exhibit significant loss in strength and thus the frequency of bleaching may be such as to severely curtail the useful life of the fabric material.

Despite the cumulative advantages inherent in the use of bleaching agents of the peroxide type, such materials present the rather serious disadvantage that maximum realization of their beneficial properties can only be obtained ordinarily with the use of elevated temperatures, i.e., temperatures in excess of about 85° C. In fact, experience establishes that temperature values of 90° C. and higher are mandatory with the use of peroxide bleaches in order to achieve the requisite degree of bleaching activity. The rather critical temperature-dependency of the peroxide and particularly the persalt bleaching agents as typified by sodium perborate poses a relatively serious drawback in view of the extensive public use of washing machines at temperatures ranging from about 50° C. to about 60° C. well below those necessary to render bleaching agents of the persalt type adequately effective for even normal household purposes. Consequently, washing operations requiring a comparatively high order of bleaching activity at reduced temperature ranges invariably necessitate resort to the use of bleaching agents other than those of the peroxide type despite the attendant disadvantages necessarily involved, e.g. with respect to

2

possible impairment of fabric strength, inferior resistance to discoloration, etc.

In order to capitalize on the advantageous features characterizing bleaching agents of the peroxide type, considerable industrial activity has centered around the research and development of means whereby to increase the effectiveness of such materials at reduced temperatures and particularly within the range of from about 50°-60° C. and, thus, to correspondingly, extend their area of effective use.

Perhaps paramount among the techniques thus far promulgated for such purposes are those based upon the use of the peroxide bleaching agent in conjunction with one or more auxiliary agents, the latter functioning as activators serving to promote or otherwise augment the bleaching capacity of the peroxide compound thereby making possible the obtention of optimum bleaching activity within the lower temperature range.

Although the precise mechanism by which activator compounds of this type function is not self-evident, it has nevertheless been postulated by way of general hypothesis that activator-peroxide interaction leads to the formation of intermediate species which function per se as bleaching agents. In a sense, then, the activator-peroxide components function together as a precursor system by which in situ generation of species providing effective bleaching means is made possible.

Although remedial techniques of the foregoing type have proved somewhat effective, it has nevertheless been ascertained in practice that the activator compounds thus far suggested in the art for such use are subject to one or more disadvantages. Perhaps the primary objection relates to the failure of such compounds to provide the desired degree of bleaching activity within the limitations imposed by economically feasible practice. Thus, it is often necessary to employ the activator in inordinately high concentrations in order to achieve satisfactory results. In other instances, it is found that the activator is not generally applicable and thus may be used advantageously solely in conjunction with specific and delimited types of peroxide bleaching agents.

Other disadvantages characterizing many of the activator compounds heretofore provided, include, for example, their incompatibility with many of the ingredients conventionally employed in formulating bleaching and/or detergent compositions. Moreover, ancillary techniques specifically devised for purposes of facilitating the required homogeneous blending of the involved ingredients have proved in many instances to be economically prohibitive, the results obtained failing to justify the concomitant increase in cost incurred.

Thus a primary object of the present invention resides in the provision of activator compounds specifically and advantageously adapted for conjoint use with peroxide compounds in bleach and/or detergent compositions wherein one or more of the disadvantages characterizing many of the compounds heretofore suggested for such purposes are eliminated, or at least alleviated to a substantial degree.

A further object of the present invention resides in the provision of activator compounds capable of augmenting the bleaching capacity of peroxide compounds to the extent of rendering such materials feasible for use in detergent and/or bleaching compositions at temperatures below about 85° C.

Another object of the present invention resides in the provision of bleaching and detergent compositions capable of yielding fabric materials having satisfactory absorbency, softness of hand and resistance to discoloration for extended periods of time under varying conditions of use.

Other objects and advantages of the present invention will become more apparent hereinafter as the description proceeds.

The attainment of the foregoing and related objects is made possible in accordance with the present invention which in its broader aspects includes the provision of activator compounds beneficially adapted for use in conjunction with peroxide bleaching agents, said activator compounds comprising water soluble chloroformates selected from the group consisting of alkyl and aryl chloroformates.

The chloroformate derivatives contemplated for use in accordance with the present invention may, for convenience, be represented according to the following structural formula:



wherein R represents alkyl and preferably lower alkyl of from 1 to 4 carbon atoms e.g. methyl, ethyl, propyl, isobutyl, etc. and aryl e.g. phenyl. It will be understood that other substituent groups may be present as integral components of the activator molecule, the primary requirement with respect thereto being that such substituents be of an innocuous nature i.e. devoid of any tendency to impair or otherwise deleteriously affect fabric materials or alternatively, to retard or otherwise interfere with the desired activator-bleaching agent interaction leading to the in situ generation of bleaching species. Suitable substituents in this regard include, for example, halogen e.g. chloro, bromo, etc.

Particularly beneficial results are obtained with the use of compounds of the above formula wherein R represents methyl, ethyl, and phenyl respectively i.e., methyl chloroformate, ethylchloroformate, and phenylchloroformate.

The chloroformate derivatives of the present invention are well known compounds with methods for their preparation being described in the published prior art, both patent and otherwise. In this connection reference is made to, for example, Dumas, Peligot—Annales de Chimie et de Physique [2], 58, 52; ibid 54, 226 and Kempf, Journal für Praktische Chemie, [2], 1, 403.

The chloroformate activators described herein are uniformly characterized in possessing outstanding capacity to augment the bleaching activity of peroxide compounds. This, of course, provides the salient advantage that the beneficial properties uniquely typical of the more mildly-acting peroxide bleaching agents such as typified by the perborates e.g. sodium perborate, are made possible at temperature ranges conventionally employed in home laundering operation. A further advantage accrues from the fact that bleaching and/or detergent composition formulated with the chloroformate activator are devoid of any tendency to weaken or otherwise deleteriously affect the strength of the fabric or textile material treated therewith, the term "textile" being used herein to connote synthetic fibers as well as products manufactured therewith. The importance of this aspect cannot be overemphasized, since the useful life of the fabric material depends critically thereupon. Thus, the compositions of the present invention may be utilized in connection with the bleaching and washing of cellulose as well as synthetic fibers such as polyamides without risk of fabric impairment. Of equal importance is the fact that the compositions described herein exhibit negligible tendency, if any, to attack the colorant present in the fiber. In addition, it is observed that the washed fabric material displays superior resistance to discoloration i.e., any yellowing tendency is not evident, while sustaining a high degree of whiteness over extended periods of time and use. The aforescribed properties rebound to particular advantage in connection with the washing and/or bleaching of cotton goods as well as other fabrics customarily employed in the manufacture of personal wearing apparel. A further advantage relates to the fact that the chloroformate activator in combination with perborate bleaching agents in particular, affords to the user

great latitude in determining and thus controlling the level of bleaching activity. This may be readily achieved in view of the comparatively mild bleaching action of the peroxides. Thus, any possibility of over-bleaching is minimized despite significant variations in the concentration of peroxide.

The chloroformate activators of the present invention may be effectively employed either singly or in admixtures comprising two or more. The efficacy of a given manner of proceeding depends primarily upon the existing requirements i.e., the specific problem to be negotiated by the bleach composition. In any event, optimum mixtures of chloroformates can be readily determined in a given circumstance by routine laboratory investigation. The employment of the chloroformate in admixture presents, of course, the singular advantage that the beneficial properties of a plurality of chloroformates can be obtained in a single composition.

The relative proportions of bleaching agent and chloroformate activator employed may vary over a relatively wide range depending somewhat upon the nature of the composition being formulated. In general, beneficial results are readily obtained by the use of the activator in amounts sufficient to yield a chloroformate peroxide mole ratio within the range of from about 0.01 to about 2.0 with a range of from 0.1 to 2.0 being preferred. Thus, in the case of a simple bleach composition, the involved ingredients will comprise, essentially, the chloroformate activator and peroxide. When formulating detergent compositions, the peroxide compound will usually be utilized in amounts sufficient to yield a concentration within the range of from about 1% to about 50%, weight basis, of total composition, with other ingredients including detergent, brightener, perfume, etc. It will be understood that the aforementioned limits are not critical per se but serve only to define those values found to yield optimum results for the broad spectrum of operations to which such compositions may be applied. The chloroformate activators described herein can likewise be employed to outstanding advantage in combination with one or more of the conventional activator compounds currently available commercially. Again, the choice of particular systems as well as concentrations lies largely within the discretion of the manufacturer. In any event, it is preferred that the chloroformate compound be used in major proportions in those instances wherein activator mixtures are employed.

As mentioned hereinbefore, the activator/bleaching agent system may be formulated together in a built detergent composition or alternatively as a separate bleach product. When provided in the latter form, the activator and bleach may be either intimately mixed or included in separate compartments of a water soluble film packet. Any of the usual methods for providing the normally liquid activator compound in powder or other suitable solid form may be resorted to for such purposes, e.g. encapsulation.

The following examples are given for purposes of illustration only and are not to be considered as necessarily limiting the subject invention. In each of the examples, the following procedure is observed. A series of washing compositions is prepared in tergotometer buckets by dissolving in 1,000 ml. of water 2 grams of a detergent of the following composition:

|                                                                                          | Percent |
|------------------------------------------------------------------------------------------|---------|
| Linear tridecyl benzene sulfonate sodium salt                                            | 21      |
| Sodium sulfate                                                                           | 26.4    |
| 65 Phosphates, tripolyphosphate, sodium tri-sodium-ortho-phosphate pyrophosphate, sodium | 35      |
| Sodium silicate                                                                          | 7       |
| Carboxymethylcellulose                                                                   | 0.4     |

70 with the remainder comprising antioxidant, perfume, etc. To each of the tergotometer buckets is added two millimoles each of sodium perborate and chloroformate activator specified so as to yield a concentration of  $2 \times 10^{-3}$  M. Control samples are similarly prepared but omitting the activator. The wash samples comprise grape-stained cotton

swatches. All washes are conducted at a temperature of 120° F. for 10 minutes followed by rinsing and air drying. The average reflectance unit reading (Rd) is determined both before and after washing and the difference between such measurements, represented in the table by  $\Delta$ Rd, for each of the systems set forth. The results obtained are itemized in the following table:

TABLE

| Ex. No. | Activator                                 | $\Delta$ Rd |
|---------|-------------------------------------------|-------------|
| 1       | Perborate (control)                       | 38.0        |
| 2       | Sodium perborate plus methylchloroformate | 49.6        |
| 3       | Sodium perborate plus ethylchloroformate  | 51.3        |
| 4       | Sodium perborate plus phenylchloroformate | 47.7        |

As the above examples make manifestly clear, the significant increase in  $\Delta$ Rd for those cotton samples treated with the alkyl chloroformate activator-perborate systems indicates that a highly efficient and active bleaching function obtained when compared to the control sample subjected to the bleaching action of the perborate alone absent the activator additive. As will be appreciated, the reflectance for a given material is a direct function of its degree of whiteness; thus, greater difference in the  $\Delta$ Rd value are indicative of correspondingly higher bleaching activity.

As mentioned hereinbefore, the composition containing the chloroformate activators described herein can be provided in the form of a bleaching composition or alternatively in the form of a built detergent product. Organic detergents suitable for use in accordance with the present invention encompass a relatively wide range of materials and may be of the anionic, non-ionic, cationic or amphoteric types.

The anionic surface active agents includes those surface active or detergent compounds which contain an organic hydrophobic group and an anionic solubilizing group. Typical examples of anionic solubilizing groups are sulfonate, sulfate, carboxylate, phosphonate and phosphate. Examples of suitable anionic detergents which fall within the scope of the invention include the soaps, such as the water-soluble salts of higher fatty acids or rosin acids, such as may be derived from fats, oils and waxes of animal, vegetable or marine origin, e.g., the sodium soaps of tallow, grease, coconut oil, tall oil and mixtures thereof; and the sulfated and sulfonated synthetic detergents, particularly those having about 8 to 26, and preferably about 12 to 22, carbon atoms to the molecule.

As examples of suitable synthetic anionic detergents there may be cited the higher alkyl mononuclear aromatic sulfonates such as the higher alkyl benzene sulfonates containing from 10 to 16 carbon atoms in the alkyl group in a straight or branched chain, e.g., the sodium salts of decyl, undecyl, dodecyl (lauryl), tridecyl, tetradecyl, pentadecyl, or hexadecyl benzene sulfonate and the higher alkyl toluene, xylene and phenol sulfonates; alkyl naphthalene sulfonate, ammonium diethyl naphthalene sulfonate, and sodium dinonyl naphthalene sulfonate.

Other anionic detergents are the olefin sulfonates, including long chain alkene sulfonates, long chain hydroxy-alkane sulfonates or mixtures of alkenesulfonates and hydroxyalkanesulfonates. These olefin sulfonate detergents may be prepared, in known manner, by the reaction of  $\text{SO}_3$  with long chain olefins (of 8-25, preferably 12-21 carbon atoms) of the formula  $\text{RCH}=\text{CHR}_1$ , where R is alkyl and  $\text{R}_1$  is alkyl or hydrogen, to produce a mixture of sultones and alkenesulfonic acids, which mixture is then treated to convert the sultones to sulfonates. Examples of other sulfate or sulfonate detergents are paraffin sulfonates, such as the reaction products of alpha olefins and bisulfites (e.g. sodium bisulfite), e.g. primary paraffin sulfonates of about 10-20, preferably about 15-20, carbon atoms; sulfates of higher alcohols; salts of  $\alpha$ -sulfofatty esters (e.g. of about 10-20 carbon atoms, such as methyl- $\alpha$ -sulfomyristate or  $\alpha$ -sulfotallowate).

Examples of sulfates of higher alcohols are sodium

lauryl sulfate, sodium tallow alcohol sulfate. Turkey red oil or other sulfated oils, or sulfates of mono- or diglycerides of fatty acids (e.g. stearic monoglyceride monosulfate), alkyl poly (ethenoxy) ether sulfates such as the sulfates of the condensation products of ethylene oxide and lauryl alcohol (usually having 1 to 5 ethenoxy groups per molecule); lauryl or other higher alkyl glyceryl ether sulfonates; aromatic poly (ethenoxy) ether sulfates such as the sulfates of the condensation products of ethylene oxide and nonyl phenol (usually having 1 to 20 oxyethylene groups per molecule preferably 2-12).

The suitable anionic detergents include also the acyl sarcosinates (e.g. sodium lauroylsarcosinate) the acyl esters (e.g. oleic acid ester) of isothionates, and the acyl N-methyl taurides (e.g. potassium N-methyl lauroyl- or oleyl tauride).

The most higher preferred water soluble anionic detergent compounds are the ammonium and substituted ammonium (such as mono-, di- and triethanolamine), alkali metal (such as sodium and potassium) and alkaline earth metal (such as calcium and magnesium) salts of the higher alkyl sulfates, and the higher fatty acid monoglyceride sulfates. The particular salt will be suitably selected depending upon the particular formulation and the proportions therein.

Nonionic surface active agents include those surface active or detergent compounds which contain an organic hydrophobic group and a hydrophilic group which is a reaction product of a solubilizing group such as carboxylate, hydroxyl, amido or amino with ethylene oxide or with the polyhydration product thereof, polyethylene glycol.

As examples of nonionic surface active agents which may be used there may be noted the condensation products of alkyl phenols with ethylene oxide, e.g., the reaction product of isoctyl phenol with about 6 to 30 ethylene oxide units; condensation products of higher fatty alcohols such as tridecyl alcohol with ethylene oxide; ethylene oxide addends of monoesters of hexahydric alcohols and inner ethers thereof such as sorbitan, mono-laurate, sorbitol mono-oleate and mannitan monopalmitate, and the condensation products of polypropylene glycol with ethylene oxide.

Cationic surface active agents may also be employed. Such agents are those surface active detergent compounds which contain an organic hydrophobic group and a cationic solubilizing group. Typical cationic solubilizing groups are amine and quaternary groups.

As examples of suitable synthetic cationic detergents there may be noted the diamines such as those of the type  $\text{RNHC}_2\text{H}_4\text{NH}_2$  wherein R is an alkyl group of about 12 to 22 carbon atoms, such as N-2-aminoethyl stearyl amine and N-2-aminoethyl myristyl amine; amide-linked amines such as those of the type  $\text{R}^1\text{CONHC}_2\text{H}_4\text{NH}_2$  wherein  $\text{R}^1$  is an alkyl group of about 9 to 20 carbon atoms, such as N-2-amino ethyl-stearyl amide and N-amino ethyl myristyl amide; quaternary ammonium compounds wherein typically one of the groups linked to the nitrogen atom is an alkyl group of about 12 to 18 carbon atoms and three of the groups linked to the nitrogen atom are alkyl groups which contain 1 to 3 carbon atoms, including such 1 to 3 carbon alkyl groups bearing inert substituents, such as phenyl groups, and there is present an anion such as halogen, acetate, methosulfate, etc. Typical quaternary ammonium detergents are ethyl-dimethyl-stearyl ammonium chloride, benzyl-dimethyl-stearyl ammonium chloride, trimethyl stearyl ammonium chloride, trimethyl-cetyl ammonium bromide, dimethyl-ethyl di-lauryl ammonium chloride, dimethyl-propyl-myristyl ammonium chloride, and the corresponding methosulfates and acetates.

Examples of suitable amphoteric detergents are those containing both an anionic and a cationic group and a hydrophobic organic group, which is advantageously a

higher aliphatic radical, e.g. of 10-20 carbon atoms. Among these are the N-long chain alkyl aminocarboxylic acids



the long chain alkyl iminodcarboxylic acids



where R is a long chain alkyl group, e.g. of about 10-20 carbons, R' is a divalent radical joining the amino and carboxyl portions of an amino acid (e.g. an alkylene radical of 1-4 carbon atoms), M is hydrogen or a salt-forming metal, R<sup>2</sup> is a hydrogen or another monovalent substituent (e.g. methyl or other lower alkyl), and R<sup>3</sup> and R<sup>4</sup> are monovalent substituents joined to the nitrogen by carbon-to-nitrogen bonds (e.g. methyl or other lower alkyl substituents). Examples of specific amphoteric detergents are N-alkyl-beta-aminopropionic acid; N-alkyl-beta-iminodipropionic acid, and N-alkyl, N,N-dimethyl glycine; the alkyl group may be, for example, that derived from coco fatty alcohol, lauryl alcohol, myristyl alcohol (or a lauryl-myristyl mixture), hydrogenated tallow alcohol cetyl, stearyl, or blends of such alcohols. The substituted aminopropionic and iminodipropionic acids are often supplied in the sodium or other salt forms, which may likewise be used in the practice of this invention. Examples of other amphoteric detergents are the fatty imidazolines such as those made by reacting a long chain fatty acid (e.g. of 10 to 20 carbon atoms) with diethylene triamine and monohalocarboxylic acids having 2 to 6 carbon atoms, e.g. 1-coco - 5 - hydroxethyl-5-carboxymethylimidazoline; betaines containing a sulfonic group instead of the carboxylic group without an intervening nitrogen atom, e.g. inner salts of 2-trimethylamino fatty acids such as 2-trimethylaminolauric acid, and compounds of any of the previously mentioned types but in which the nitrogen atom is replaced by phosphorus.

The detergent composition may further contain one or more water-soluble builder salts which may be either organic or inorganic in nature. Suitable representatives include the following:

Trisodium phosphate,  
Tetrasodium pyrophosphate,  
Sodium acid pyrophosphate,  
Sodium tripolyphosphate,  
Sodium monobasic phosphate,  
Sodium dibasic phosphate,  
Sodium hexametaphosphate,  
Sodium silicates, Na<sub>2</sub>O/SiO<sub>2</sub> of 1/1.6 to 1/3.2  
Sodium carbonate,  
Sodium sulfate,  
Borax,  
Ethylene diamine tetraacetic acid tetrasodium salts, etc.

Mixtures of two or more inorganic or organic salts can be used, as can mixtures of inorganic and organic salts.

Particularly preferred herein are water-soluble, alkali metal polyphosphate builder salts. These salts form water-soluble complexes with calcium and magnesium ions found in hard water and thereby prevent the formation of insoluble salts which tend to deposit upon textiles during a washing cycle. Further, such phosphates enhance the detergency efficiency of anionic detergents, aid in controlling sudsing and powers and aid in keeping soil suspended in the washing bath after its removal from the soiled textiles.

Various other materials may be included in compositions of the invention, whether in solid or liquid form, by addition in a known manner to the aqueous mixtures or to the solidified product. Examples thereof are the higher fatty acid amides such as coconut or lauric mono-

ethanolamide, isopropanolamide and the like; hydroscopic solubilizing agents such as xylene or toluene sulfonates; organic solubilizing agents such as ethanol, ethylene glycol and hexylene glycol; sodium carboxymethylcellulose and polyvinyl alcohol antiredeposition agents; optical and fluorescent brightener materials; coloring agents; corrosion inhibiting agents; germicides; perfumes, bluing agents; and the like.

Preferred compositions advantageously contain a hydrophobic colloidal cellulosic soil-suspending agent which is soluble or dispersible in water also. The joint use of the combination of the cellulosic compound and polyvinyl alcohol is particularly effective for soil-suspension properties during the washing of a variety of fabrics, including both cotton and synthetic fibers such as nylon, Dacron, and resin-treated cottons. The mixtures are used preferably in a total amount of 0.1 to 2 percent by weight of the solids. Preferred cellulosic compounds are the alkali metal salts of a carboxy lower alkyl cellulose having up to 3 carbons in the alkyl group, such as the sodium and potassium salt of carboxymethylcellulose. Suitable salts are sodium carboxyethylcellulose; the cellulose sulfates and lower alkyl and hydroxyalkylcellulose ethers such as methyl-, ethyl-, and hydroxyethylcellulose.

The proportions of such ingredients are not particularly critical and may be selected in accordance with usual practice. Thus, for example, the organic detergent may be employed in concentrations ranging from about 2% and preferably from about 10% to about 50% by weight of the composition. The builder salts, whether organic or inorganic, are preferably employed in concentrations ranging from about 10% to about 95% by weight of the composition. Exemplary of bleaching formulations capable of providing the improvements described herein include a composition comprising sodium carbonate (5 parts), sodium tripolyphosphate (30 parts), ethyl chloroformate (15.5 parts), sodium perborate (22 parts), alkylbenzenesulfonate (2 parts), with the remainder comprising on a 100 parts basis sodium sulfate, brightener, perfume, chelating agent, etc. It will be understood that the foregoing composition is given solely for purposes of illustration; thus, departures from the specific concentrations stipulated may be dictated in a particular circumstance depending upon the specific requirements of the user.

Results similar to those described in the foregoing examples are obtained when the procedures delineated therein are repeated but employing in lieu of sodium perborate, equivalent concentrations of one or more of sodium percarbonate, sodium persilicate, etc. The terminology "water-soluble peroxide," "persalt" bleaching agent as used herein is intended to connote those compounds which give use to hydrogen peroxide when dissolved in water. Thus, the peroxide compounds hereinbefore described as being suitable in the practice of the present invention are believed to contain hydrogen peroxide of crystallization.

The bleaching and detergent compositions of the present invention entail the further advantage that they may be effectively employed over a relatively wide pH range in the virtual absence of risk of damage to the fabric material. The desired pH may be readily obtained by the addition of suitable buffering agents to the bleaching solution. Moreover, the effectiveness of the bleaching or detergent composition at relatively high pH permits their advantageous use in combination with common household laundry soaps and detergents for preventive bleaching of fiber materials. In any event, a pH within the range of from about 6-10 is recommended for the vast majority of bleaching and washing applications.

The present invention has been described with respect to certain preferred embodiments thereof and there will become obvious to persons skilled in the art other variations, modifications, and equivalents which are to be understood as coming within the scope of the present invention.

## What is claimed is:

1. A process of bleaching textiles comprising the steps of placing the textiles to be bleached in an aqueous solution of water-soluble, inorganic peroxide bleaching agent and a water-soluble chloroformate selected from the group consisting of C<sub>1</sub>-C<sub>4</sub> alkyl and phenyl chloroformates wherein the chloroformate peroxide mole ratio ranges from about .01 to about 2.0, allowing the textiles to remain in the solution for a normal washing period and rinsing the textiles.

2. A process as described in claim 1 wherein included in the aqueous solution is a water-soluble, organic detergent selected from the group consisting of anionic, cationic, nonionic, and amphoteric detergents.

## References Cited

## UNITED STATES PATENTS

- |   |           |         |                          |         |
|---|-----------|---------|--------------------------|---------|
| 5 | 2,955,905 | 10/1960 | Davies et al. -----      | 8—111   |
|   | 3,130,165 | 4/1964  | Brocklehurst et al. ---- | 282—99  |
|   | 3,332,882 | 7/1967  | Blumbergs et al. -----   | 252—186 |

MAYER WEINBLATT, Primary Examiner

U.S. Cl. X.R.

252—95, 186